

# United States Patent [19]

Christiansen et al.

[11] 3,907,632

[45] Sept. 23, 1975

[54] BLEACHING CELLULOSIC PULPS WITH  
GASEOUS CHLORINE AT A pH OF 7 TO 10  
IN A MULTISTAGE BLEACHING PROCESS

[75] Inventors: Claud B. Christiansen; William R.  
Dial, both of Akron, Ohio

[73] Assignee: PPG Industries, Inc., Pittsburgh, Pa.

[22] Filed: Oct. 23, 1973

[21] Appl. No.: 408,770

[52] U.S. Cl. 162/66; 162/88; 162/89

[51] Int. Cl.<sup>2</sup> D21C 9/12

[58] Field of Search 162/89, 66, 88

[56] References Cited

UNITED STATES PATENTS

2,968,589 1/1961 Saunders et al. 162/89 X

3,433,702 3/1969 Jack et al. 162/88 X  
3,501,374 3/1970 Jack et al. 162/89  
3,579,419 5/1971 Yorston et al. 162/66  
3,586,599 6/1971 Yorston et al. 162/88 X  
3,619,349 11/1971 Liebergott et al. 162/66  
3,630,828 12/1971 Liebergott et al. 162/66 X

Primary Examiner—S. Leon Bashore

Assistant Examiner—Arthur L. Corbin

Attorney, Agent, or Firm—Mark Levin

[57] ABSTRACT

This invention relates to multistage bleaching of cellulosic pulp wherein gaseous chlorine is contacted with cellulosic pulp at high consistency in the third or subsequent stage of a multistage bleaching process, while maintaining the pH of the pulp between about 7 and about 10.

17 Claims, No Drawings

**BLEACHING CELLULOSIC PULPS WITH  
GASEOUS CHLORINE AT A PH OF 7 TO 10 IN A  
MULTISTAGE BLEACHING PROCESS**

**STATE OF THE ART**

In the multistage bleaching of an unbleached chemical cellulosic pulp, i.e. wood pulp, the pulp from the digestion stage in, for example, the kraft, soda, or sulfite process, normally after washing, is treated to render at least a portion of the ligneous impurities readily soluble in water or soluble in dilute aqueous alkali, such as dilute aqueous solutions of sodium hydroxide, sodium sulfite or ammonium hydroxide. To accomplish this solubilization of ligneous impurities, the pulp is conventionally treated with agents such as chlorine, chlorine dioxide, or the oxides of nitrogen, more usually chlorine or chlorine dioxide. This process which is more a purification step or pretreatment step rather than a true bleaching step is generally considered the first stage in a multistage pulp bleaching process.

After the first stage treatment, the pulp, after washing with water, is subjected to alkaline extraction with, for example, sodium hydroxide to remove water insoluble ligneous impurities. The extraction is generally conducted on the pulp at low consistency in the range of 10 to 14%, a temperature range of 40° to 70°C. and at a retention time of about 1 to 2 hours. This sequence is generally considered the second stage of a multistage bleaching process.

Subsequent to the basic extraction stage and normally after water washing, the pulp is subjected to a bleaching or oxidizing stage, which is normally considered the third stage in a multistage bleaching process.

The preceding three stages are present in essentially all multistage bleaching processes for chemical cellulosic pulps although variations are possible. For example, with pulp made from certain wood species, treatment with sodium or calcium hypochlorite may be desirable between the stage two extraction and third stage oxidative or bleach treatment. Further, with certain pulps, especially where high brightness is desired, there is employed an additional fifth bleaching or oxidizing stage which is not infrequently similar to the third stage. These two oxidizing or bleaching stages are separated by a fourth stage, a basic extraction procedure similar to the second stage. This five stage bleaching process is commonly utilized with kraft pulps.

The use of chlorine in various forms in the treatment of chemical pulps has been described in the art.

Canadian Pat. No. 886,479 describes treating high consistency pulps with high concentrations of chlorine gas or gaseous chlorine dioxide mixtures for relatively short times. The treatment may be conducted in a chlorination, extraction, chlorination, extraction sequence.

U.S. Pat. No. 3,433,702 generally describes the use of aqueous or gaseous chlorine in various stages of pulp bleaching and is drawn to a process wherein low consistency pulps are bleached in a sequence wherein pulp is first reacted with chlorine dioxide until the chlorine dioxide is at least partially depleted. The pulp is then reacted with chlorine.

U.S. Pat. No. 3,707,436 describes a process wherein pulp fiber is exploded or expanded. An aqueous solution of the fiber is then subjected to two chlorination stages wherein aqueous or gaseous chlorine may be employed.

U.S. Pat. No. 3,560,330 describes bleaching low consistency pulps with chlorine with relatively long chlorination times.

U.S. Pat. No. 2,166,330 describes the use of mixtures of chlorine and chlorine dioxide to avoid fiber degradation.

U.S. Pat. No. 3,619,349 describes bleaching high consistency pulps with gaseous chlorine monoxide in a multistage bleaching process.

**DESCRIPTION OF THE INVENTION**

It has now been found that significant benefits can be obtained in bleaching a chemical cellulosic pulp, by employing a novel bleaching step in at least one stage subsequent to the initial steps of solubilizing ligneous impurities and followed by extraction with a base, in a multistage bleaching process.

The novel process step comprises accomplishing bleaching of the resultant fibrous cellulosic pulp in a third or subsequent step in the multistage bleaching process by contacting the pulp at a high consistency and in the form of fluffed or shredded fibers and fiber aggregates with gaseous chlorine.

In particular, it has been found that in the bleaching of chemical cellulosic pulps in the gaseous phase at high consistency and in fluffed and shredded form, chlorine can be used with advantage in those stages of a multistage bleaching process where chlorine dioxide or chlorine monoxide have been used to achieve a similar oxidative bleaching effect.

The use of gaseous chlorine presents several distinct advantages, the first being safety. Both chlorine dioxide and chlorine monoxide tend to form explosive mixtures which create safety hazards. The handling of chlorine presents a significantly lower safety hazard in this regard. Cost is another significant factor, both the use of chlorine dioxide and chlorine monoxide require facilities for their preparation, and which thereof add to the cost of the process and further which can introduce variables into their use.

Further, the use of gaseous chlorine presents significant time and temperature advantages over the use of chlorine dioxide. It has been found that in the bleaching of a chemical cellulosic pulp, particularly wood pulp, such as a kraft or sulfite pulp, at high consistency by contacting with gaseous chlorine, it is possible to achieve substantial improvements in Elrepho brightness within 1 to 5 minutes where a typical gaseous chlorine dioxide treatment requires 30 minutes.

In a particularly preferred embodiment, gaseous chlorine is employed in a high consistency bleaching stage subsequent to an intermediate bleaching stage employing chlorine dioxide; for example, in the fifth stage of a process which involves subjecting chemical pulp to chlorination extraction, chlorine dioxide, extraction, with a fifth stage being the contacting of the resultant pulp at high consistency with gaseous chlorine as described herein.

The process of the invention is equally applicable to pretreated or prebleached pulps having a relatively low Permanganate Number (TAPPI Standard T-214), which are items of commerce. These are chemical cellulosic pulps which have been subjected to pretreatment or prebleaching, for example, by subjection to the first two stages of a conventional multistage bleaching process, and have had at least a significant portion of their ligneous constituents removed. For example, the process of the invention is useful in bleaching virtually

any partially bleached chemical cellulosic pulp preferably having a Permanganate Number less than about 5 and preferably less than above 3.

The pulp contacted with gaseous chlorine in the process of the invention is a high consistency pulp, that is a pulp which is essentially free of a continuous aqueous phase. Generally, high consistency pulps contain at least about 15% fibers on a moisture-free fiber basis. Preferably, the pulps employed have a consistency of about 15 to about 50%. It is desirable that the pulp have a consistency of about 15 to about 35%. The primary criteria for distinguishing high consistency pulp from low consistency pulp, that is pulp which is a slurry of fibers in a discrete aqueous phase, is the substantial absence of a discrete liquid aqueous phase. Otherwise stated, in high consistency pulp substantially all water present is retained by the fibers so that there can be created a shredded and fluffed material which has a large surface area in contact with the surrounding atmosphere.

In the process of the invention, gaseous chlorine is fed into a bleaching zone containing cellulosic pulp at high consistency to thereby induce bleaching. This bleaching zone may take the form of a batch reactor or a continuous reactor where the pulp and chlorine are charged in either a countercurrent or concurrent fashion with means to provide adequate contacting of the charged materials. The mechanism of bleaching is not fully known and while gaseous chlorine is fed into the bleaching zone, it may, in fact, be transformed, for example, at the gas-pulp interface, or in or on the fiber, at least in part, to at least one other chemical moiety which may, in fact, be the actual bleaching moiety.

The fluffed high consistency pulp can be contacted with a gaseous feed which is essentially 100% chlorine, devoid of intentionally added amounts of chlorine monoxide, for example, i.e. essentially pure chlorine gas, or the chlorine may be diluted with a non-reactive gas such as air, carbon dioxide or nitrogen, to provide a gaseous medium wherein the active contacting component consists essentially of gaseous chlorine. Typically, when a non-reactive gas diluent is employed, the chlorine is diluted with such a gas in the range of about 4:1 to 1:4. The use of a pure chlorine-containing gas is in contrast to the use of chlorine monoxide or chlorine dioxide which is diluted for safe usage.

To aid in the distribution of the chlorine throughout the pulp, it is preferred that the pulp be agitated during or after the introduction of the desired amount of chlorine into the bleaching zone. This agitation may be accomplished by tumbling or other appropriate means.

The amount of chlorine added is subject to wide variation and obviously the history of the pulp, including the length and severity of prior treatments, governs the amount of chlorine necessary to achieve optimum results. Surprisingly, it has been found, however, that the introduction of low amounts of chlorine below 2% by weight of chlorine based on moisture-free fiber into the bleaching zone accomplishes substantial bleaching. Typically, the use of chlorine in an amount of about 1% by weight or less based on the moisture-free fiber provided highly effective bleaching, such as that achieved by the use of chlorine dioxide or chlorine monoxide. While the use of higher amounts of chlorine provide effective bleaching, when higher amounts of chlorine are employed, fiber viscosities tend to be lowered.

The temperature at the time of contact between the pulp and the gaseous chlorine is not particularly critical

in achieving a bleaching effect. It is preferred that the temperature in the contacting zone be at about room temperature. Bleaching is rapidly accomplished at ambient temperature and, while elevated temperature can be employed, heating is unnecessary and the use of elevated temperatures tend to reduce fiber viscosity.

The pH maintained in the process has a significant effect on the viscosity of the pulp obtained. It has been found desirable to maintain the pH of the pulp at a pH which is at least about neutral or alkaline during the process of the invention. Typically at the end of the gaseous chlorine contacting step, as measured as hereinafter described, is between about 7 and about 10 and preferably between about 7 and about 9. The pH of the reaction mixture may be positively controlled by several means. Since the pulp treated by the process of the invention has been previously subjected to alkaline extraction, the amount of subsequent washing may be controlled so that sufficient base remains in the fibers to maintain the pH in the desired range throughout the gaseous chlorine contacting step. Another method of controlling the pH comprises adding to the pulp, prior to contacting the pulp with gaseous chlorine or incrementally during the contacting of the pulp with gaseous chlorine, sufficient base to maintain the pH in the desired range through the gaseous chlorine contacting step. The base employed can vary widely since its primary function is pH maintenance. Strong bases, such as sodium hydroxide and the like, may be employed. Relatively weak bases, such as ammonium hydroxide and the like, are equally operable. Where it is desirable to maintain the highest possible fiber viscosities, it has been found desirable to employ a buffering agent, such as an alkali metal salt of a weak acid; for example, sodium carbonate, may be employed. The alkali metal carbonates, such as sodium carbonate, sodium bicarbonate, either hydrous or anhydrous, and the like, are highly useful.

Since the direct measurement of the pH of the high consistency pulp is difficult, since essentially no free aqueous phase is present, pH is measured by diluting the high consistency pulp with water to form a low consistency pulp with a consistency of about 7%, and measuring the pH of the aqueous phase so produced.

The reaction time necessary to achieve substantial bleaching effect is relatively short. The substantial portion of the bleaching effect occurs in the first 1 to 5 minutes of contact time between the high consistency fluffed pulp and the gaseous chlorine, while contact may be continued for up to 30 minutes or even an hour, such time periods are generally not necessary and may contribute to fiber viscosity degradation.

The invention is further described in the following examples which are to be considered illustrative rather than limiting. All parts and percentages are by weight unless otherwise specified.

#### EXAMPLE 1

This example shows the use of chlorine to bleach high consistency pulp in the fifth stage of a multistage bleaching process. The pulp treated was a softwood kraft pulp having an unbleached K number of 14.9 (Permanganate No. TAPPI Standard T-214) and a cupriethylenediamine (CED) 0.5% viscosity of 18.4 centipoise (TAPPI T-230).

The pulp was pretreated, in the conventional manner, with a first stage chlorination step at 3% consistency by contacting the pulp with chlorine water

(5.25% Cl on moisture-free fiber) at room temperature for 60 minutes. The chlorine water was then drained and the pulp thoroughly washed with water.

The chlorination step was followed by a second stage extraction step wherein the pulp at 12% consistency was contacted with 10% sodium hydroxide (3% sodium hydroxide on moisture-free fiber) at 165°F. for 90 minutes. The caustic solution was drained and the pulp thoroughly washed with water.

The resultant pulp at 12% consistency was then bleached with chlorine dioxide, by heating the pulp to 165°F. and adding 0.5% chlorine dioxide (7 gm/liter solution in water) and holding the mixture at 165°F. for 2 hours, drained and thoroughly washed with water.

The resultant pulp was then subjected to a fourth stage extraction step wherein the pulp at 12% consistency

cupying about half the volume of the chamber. Chlorine gas diluted with nitrogen (3 volumes of  $N_2$ /volume of  $Cl_2$ ) was passed into the bottom of the chamber and was absorbed within the fiber mass. The chamber was sealed and repeatedly (10-15 times) rapidly inverted to assure mixing by tumbling of the fibers. The chamber was then allowed to stand the remainder of the reaction time.

At the end of the reaction time, the contents of the chamber were placed in sufficient water to reduce the consistency to 7.5%, at which time, after mixing, pH was measured by squeezing the pulp in a muslin cloth to remove water and measuring the pH of the water.

The pulp was then washed with water at 120°F. and filtered. The results of the multistage treatment are set forth in Table I.

TABLE I

| Bleaching of Prebleached (CEDE) Kraft Pulp with Chlorine |                       |      |                                 |                          |            |            |          |                   |                    |
|----------------------------------------------------------|-----------------------|------|---------------------------------|--------------------------|------------|------------|----------|-------------------|--------------------|
| Run No.                                                  | Chemical, % m.f. Pulp |      |                                 | Consistency, % m.f. Pulp | Temp., °F. | Time, Min. | pH Final | CED Viscosity, cp | Elrepho Brightness |
|                                                          | Cl <sub>2</sub>       | NaOH | Na <sub>2</sub> CO <sub>3</sub> |                          |            |            |          |                   |                    |
| <b>Prebleached Kraft Pulp</b>                            |                       |      |                                 |                          |            |            |          |                   |                    |
| 1                                                        | 0.3                   | 0.10 | —                               | 30                       | 80         | 5          | 4.2      | 11.8              | 82.8               |
| 2                                                        | 0.3                   | 0.15 | —                               | 30                       | 80         | 5          | 4.5      | 11.9              | 89.5               |
| 3                                                        | 0.3                   | 0.20 | —                               | 30                       | 80         | 5          | 5.7      | 12.5              | 89.9               |
| 4                                                        | 0.3                   | 0.40 | —                               | 30                       | 80         | 5          | 7.7      | 12.0              | 91.1               |
| 5                                                        | 0.3                   | —    | 0.20                            | 30                       | 80         | 5          | 4.4      | 12.0              | 89.4               |
| 6                                                        | 0.3                   | —    | 0.25                            | 30                       | 80         | 5          | 5.4      | 12.5              | 89.8               |
| 7                                                        | 0.3                   | —    | 0.30                            | 30                       | 80         | 5          | 6.7      | 12.6              | 89.1               |
| 8                                                        | 0.3                   | —    | 0.40                            | 30                       | 80         | 5          | 7.0      | 12.8              | 90.3               |
| 9                                                        | 0.3                   | —    | 0.60                            | 30                       | 80         | 5          | 7.8      | 13.0              | 90.5               |
| 10                                                       | 0.17                  | —    | 0.20                            | 30                       | 80         | 5          | 7.1      | 13.3              | 90.8               |
| 11                                                       | 0.17                  | —    | 0.25                            | 30                       | 80         | 5          | 7.3      | 13.4              | 90.9               |
| 12                                                       | 0.17                  | —    | 0.30                            | 30                       | 80         | 5          | 7.6      | 13.3              | 90.7               |
| 13                                                       | 0.3                   | 0.10 | —                               | 30                       | 80         | 1          | 7.5      | 11.6              | 90.9               |
| 14                                                       | 0.3                   | 0.15 | —                               | 30                       | 80         | 1          | 7.6      | 12.0              | 90.6               |
| 15                                                       | 0.3                   | 0.20 | —                               | 30                       | 80         | 1          | 7.9      | 12.4              | 90.2               |
| 16                                                       | 0.30                  | 0.3  | —                               | 30                       | 80         | 1          | 6.9      | 12.1              | 90.9               |
| 17                                                       | 0.30                  | 0.4  | —                               | 30                       | 80         | 1          | 7.3      | 12.2              | 91.1               |
| 18                                                       | 0.30                  | 0.5  | —                               | 30                       | 80         | 1          | 8.4      | 12.7              | 90.7               |

tency was treated with 1% sodium hydroxide at 165°F. for 90 minutes. The pulp was then drained and washed with water.

The resultant pulp was reduced to 60-70% consistency and then shredded and fluffed in increments in a Waring Blender. The pulp was divided into portions

When aliquots of the pretreated pulp, as formed in the first four stages, fluffed and treated, as set forth above, were subjected to a fifth stage bleaching under the same conditions, but replacing chlorine with an equivalent amount of chlorine monoxide, the following results were obtained, as set forth in Table II:

TABLE II

| Bleaching of Prebleached (CEDE) Kraft Pulp with Chlorine Monoxide |                        |      |                                 |                          |            |            |          |                   |                    |
|-------------------------------------------------------------------|------------------------|------|---------------------------------|--------------------------|------------|------------|----------|-------------------|--------------------|
| Run No.                                                           | Chemical, % m.f. Pulp  |      |                                 | Consistency, % m.f. Pulp | Temp., °F. | Time, Min. | pH Final | CED Viscosity, cp | Elrepho Brightness |
|                                                                   | Equiv. Cl <sub>2</sub> | NaOH | Na <sub>2</sub> CO <sub>3</sub> |                          |            |            |          |                   |                    |
| 1                                                                 | 0.3                    | —    | —                               | 30                       | 80         | 5          | 6.1      | 13.5              | 90.7               |
| 2                                                                 | 0.3                    | 0.05 | —                               | 30                       | 80         | 5          | 6.8      | 12.7              | 91.2               |
| 3                                                                 | 0.3                    | 0.10 | —                               | 30                       | 80         | 5          | 7.4      | 12.6              | 91.4               |
| 4                                                                 | 0.3                    | —    | 0.05                            | 30                       | 80         | 5          | 6.6      | 12.5              | 91.2               |
| 5                                                                 | 0.3                    | —    | 0.10                            | 30                       | 80         | 5          | 6.5      | 11.9              | 90.6               |
| 6                                                                 | 0.3                    | —    | 0.15                            | 30                       | 80         | 5          | 6.8      | 12.1              | 90.8               |
| 7                                                                 | 0.3                    | —    | 0.30                            | 30                       | 80         | 5          | 7.5      | 12.2              | 91.2               |
| 8                                                                 | 0.17                   | —    | 0.05                            | 30                       | 80         | 5          | 6.9      | 12.6              | 90.6               |
| 9                                                                 | 0.17                   | —    | 0.10                            | 30                       | 80         | 5          | 7.3      | 12.8              | 90.8               |
| 10                                                                | 0.17                   | —    | 0.15                            | 30                       | 80         | 5          | 7.7      | 12.7              | 90.9               |

0.3% available chlorine is equivalent to 0.18% Cl<sub>2</sub>O  
0.17% available chlorine is equivalent to 0.10% Cl<sub>2</sub>O

which were treated in the following manner. The portions were sprayed with water sufficient to reduce the consistency to 30%. Where base or buffers were added to adjust pH (i.e. NaOH or Na<sub>2</sub>CO<sub>3</sub>), these were incorporated into the water sprayed upon the fluffed fibers. The fluffed fibers were placed into a glass chamber oc-

## EXAMPLE 2

This example illustrates three stage bleaching utilizing gaseous chlorine in the third stage. The pulp treated was a softwood kraft pulp which has an unbleached K number of 14.9 and a CED viscosity of 18.4 centipoise.

The pulp was treated by a first stage chlorination and a second stage caustic extraction to yield a pulp having a CED viscosity of 14.0 centipoise and an Elrepho brightness of 48.4. The third stage chlorination step was conducted as in Example 1. The results found in treating divided portions of the extracted high consistency fluffed pulp are summarized in Table III.

into a glass chamber, occupying about half the volume of the chamber. The fibers are rested upon a perforated glass grid which raises the fibers above the gas inlet in the bottom of the chamber to allow for gas circulation about the fibers. Chlorine gas diluted with nitrogen (3 volumes of  $N_2$ /volume of  $Cl_2$ ) was passed into the bottom of the chamber and absorbed within the fiber

TABLE III

| Bleaching of Pretreated (CE) Softwood Kraft Pulp with Chlorine |                       |      |                          |       |            |            |               |                    |      |
|----------------------------------------------------------------|-----------------------|------|--------------------------|-------|------------|------------|---------------|--------------------|------|
| Run No.                                                        | Chemical, % m.f. Pulp |      | Consistency, % m.f. Pulp |       | Temp., °F. | Time, Min. | CED           |                    |      |
|                                                                | $Cl_2$                | NaOH | Pulp                     | Final |            |            | Viscosity, cp | Elrepho Brightness |      |
| Pretreated Kraft Pulp                                          |                       |      |                          |       |            |            |               |                    |      |
| 1                                                              | 0.6                   | 0    | 30                       | 80    | 5          | 3.2        | 14.0          | 12.6               | 48.4 |
| 2                                                              | 0.6                   | 0.20 | 30                       | 80    | 5          | 3.9        | 12.6          | 72.5               |      |
| 3                                                              | 0.6                   | 0.40 | 30                       | 80    | 5          | 4.9        | 10.9          | 10.3               | 74.3 |
|                                                                |                       |      |                          |       |            |            | 75.0          |                    |      |

The pretreated pulp contained caustic soda left in the pulp by means of a final wash with caustic solution to obtain good distribution of buffer before fluffing.

## EXAMPLE 3

This example shows the use of gaseous chlorine to bleach high consistency pulp in the third and fifth stages of a multistage bleaching process. The pulp treated was a softwood kraft pulp having an unbleached K number of 14.9 and a CED viscosity of 15.4 centipoise.

The pulp was pretreated, in a conventional manner, with a first stage chlorination step at 3% consistency by contacting chlorine water (5% chlorine on a moisture-free pulp basis) at room temperature (75°F.) for 60 minutes. The chlorine water was then drained and the pulp thoroughly washed with water.

The chlorination step was followed by a second stage

25

mass. The chamber was sealed and repeatedly inverted to tumble the fibers. The chamber was then allowed to stand for the remainder of the reaction time.

30

The above bleaching step was followed by a fourth stage extraction step where the fibers were extracted with dilute caustic (1.0% caustic on a moisture-free fiber basis), at 12% consistency, at 165°F. for 90 minutes. The fibers were then thoroughly washed with water.

35

The fibers were then dried to above 70% consistency and treated in a fifth stage with gaseous chlorine, at 30% consistency in the same manner as the third stage.

35

The conditions and results of each of the stages, with varying conditions in the third and fifth stage gaseous chlorination steps, are set forth in Table IV.

TABLE IV

| Bleaching Softwood Kraft Pulp by Sequence CEC <sub>2</sub> EC <sub>2</sub> |           |                       |      |                          |            |            |          |               |                    |
|----------------------------------------------------------------------------|-----------|-----------------------|------|--------------------------|------------|------------|----------|---------------|--------------------|
| Run No.                                                                    | Stage No. | Chemical, % m.f. Pulp |      | Consistency, % m.f. Pulp | Temp., °F. | Time, Min. | pH Final | CED           |                    |
|                                                                            |           | $Cl_2$                | NaOH |                          |            |            |          | Viscosity, cp | Elrepho Brightness |
|                                                                            | 1         | 5.0                   | —    | 3                        | 75         | 60         | 1.8      | —             | —                  |
|                                                                            | 2         | —                     | 3.0  | 12                       | 165        | 75         | 11.4     | 12.5          | 56.6               |
| 1                                                                          | 3         | 0.6                   | 0.5  | 30                       | 82         | 5          | 7.1      | —             | —                  |
|                                                                            | 4         | —                     | 1.0  | 12                       | 165        | 90         | 11.6     | —             | —                  |
|                                                                            | 5         | 0.3                   | 0.4  | 30                       | 81         | 5          | 7.2      | 7.3           | 87.4               |
| 2                                                                          | 3         | 0.6                   | 0.6  | 30                       | 82         | 5          | 7.6      | —             | —                  |
|                                                                            | 4         | —                     | 1.0  | 12                       | 165        | 90         | 11.5     | —             | —                  |
|                                                                            | 5         | 0.3                   | 0.4  | 30                       | 81         | 5          | 7.2      | 7.4           | 88.1               |
| 3                                                                          | 3         | 0.6                   | 0.7  | 30                       | 82         | 5          | 7.8      | —             | —                  |
|                                                                            | 4         | —                     | 1.0  | 12                       | 165        | 90         | 11.6     | —             | —                  |
|                                                                            | 5         | 0.3                   | 0.4  | 30                       | 81         | 5          | 7.4      | 7.8           | 88.0               |

extraction step wherein the pulp was contacted at 12% consistency with 10% sodium hydroxide (3% sodium hydroxide on a moisture-free fiber basis) at 165°F. for 75 minutes. The caustic solution was drained and the pulp thoroughly washed with water.

The resultant pulp dried to about 70% consistency was then shredded and fluffed in increments in a Waring Blender. The pulp was divided into portions which were treated, in a third stage, in the following manner. The portions were sprayed with a fine mist of water containing sufficient sodium hydroxide to obtain the final desired pH. The fluffed fibers were then placed

60 The conditions and quantities of reagents in the above examples may be varied within the scope of the disclosure while obtaining results within the scope of this invention. Likewise, various pulps or reagents, such as those described hereinabove, may be substituted for those exemplified to obtain equivalent results.

According to the provisions of the Patent Statutes, there are described above the invention and what are now considered to be its best embodiments. However, within the scope of the appended claims, it is to be understood that the invention may be practiced otherwise than specifically described.

What is claimed is:

1. In a multistage process for bleaching a fibrous cellulosic pulp wherein the pulp has been subjected at least to a chemical treatment stage to solubilize ligneous impurities, followed by a subsequent alkaline extraction treatment, the improvement which comprises contacting the resultant pulp in at least one subsequent stage at high consistency and in the form of fluffed or shredded fibers or fiber aggregates, with a gaseous medium wherein the active bleaching contacting component consists essentially of gaseous chlorine wherein the amount of gaseous chlorine in each gaseous chlorine contacting stage is an effective bleaching inducing amount of chlorine which is about 1% or less by weight based on the weight of moisture-free cellulosic pulp and the pH of the pulp is maintained between about 7 and about 10 during the gaseous chlorine contacting stage, thereby effecting a bleaching of said pulp.

2. In a multistage process for bleaching a fibrous cellulosic pulp wherein the pulp has been subjected at least to a chemical treatment stage to solubilize ligneous impurities, followed by a subsequent alkaline extraction treatment, the improvement which comprises contacting the resultant pulp in at least one subsequent stage at high consistency and in the form of fluffed or shredded fibers or fiber aggregates with a gaseous medium wherein the active contacting component consists essentially of gaseous chlorine wherein the amount of gaseous chlorine in each gaseous chlorine contacting stage is an effective bleaching inducing amount of chlorine which is about 1% or less by weight based on the weight of moisture-free cellulosic pulp, thereby effecting bleaching of said pulp, where the pulp prior to contacting with chlorine has been subjected to an alkaline extraction stage wherein the amount of residual base in the pulp at the termination of the extraction stage is controlled to provide a pH of between about 7 and about 10 at the termination of the gaseous chlorine contacting stage.

3. In a multistage process for bleaching a fibrous cellulosic pulp wherein the pulp has been subjected at least to a chemical treatment stage to solubilize ligneous impurities, followed by a subsequent alkaline extraction treatment, the improvement which comprises contacting the resultant pulp in at least one subsequent stage at high consistency and in the form of fluffed or shredded fibers or fiber aggregates with a gaseous medium wherein the active contacting component consists essentially of gaseous chlorine wherein the amount of gaseous chlorine in each gaseous chlorine contacting stage is an effective bleaching inducing amount of chlorine which is about 1% or less by weight based on the weight of moisture-free cellulosic pulp, thereby effecting bleaching of said pulp, sufficient base being added to the gaseous chlorine contacting stage to maintain the pH in the gaseous chlorine contacting stage between about 7 and about 10.

4. A process, as in claim 3, wherein the base is an alkali metal salt of a weak acid.

5. In a multistage process for bleaching a fibrous cellulosic pulp wherein the pulp has been subjected at least to a chemical treatment stage to solubilize ligneous impurities, followed by a subsequent alkaline extraction treatment, the improvement which comprises contacting the resultant pulp in at least one subsequent stage at high consistency and in the form of fluffed or shredded fibers or fiber aggregates with a gaseous medium wherein the active contacting component consists

essentially of gaseous chlorine wherein the amount of gaseous chlorine in each gaseous chlorine contacting stage is an effective bleaching inducing amount of chlorine which is about 1% or less by weight based on the weight of moisture-free cellulosic pulp, thereby effecting bleaching of said pulp, sufficient amounts of an alkali metal carbonate being added to the gaseous chlorine contacting stage to maintain the pH in the gaseous chlorine contacting stage between about 7 and 10.

6. A process, as in claim 3, wherein the base is sodium hydroxide.

7. A process, as in claim 1, wherein the high consistency pulp has a consistency between about 15 and about 50.

8. In a process of bleaching a cellulosic pulp which comprises:

- treating a chemical cellulosic pulp in a first stage to solubilize ligneous impurities,
- extracting the resultant pulp with aqueous base,
- bleaching the resultant pulp with chlorine dioxide, and
- extracting the resultant pulp with aqueous base, the improvement which comprises,
- contacting the resultant pulp at high consistency and in the form of fluffed or shredded fibers or fiber aggregates with a gaseous medium wherein the active contacting component consists essentially of gaseous chlorine wherein the amount of gaseous chlorine is an effective bleaching inducing amount of chlorine which is about 1% or less by weight based on the weight of moisture-free cellulosic pulp, while the pH of the pulp is maintained between about 7 and about 10 during the gaseous chlorine contacting stage, thereby effecting bleaching of said pulp.

9. A process, as in claim 8, wherein the pulp prior to contact with chlorine has been subjected to a basic extraction stage and wherein the amount of residual base in the pulp at the termination of the extraction stage is controlled to provide the desired pH in the gaseous chlorine contacting stage.

10. A process, as in claim 8, wherein a pH maintaining amount of base is added to the pulp prior to the gaseous chlorine contacting stage.

11. A process, as in claim 10, wherein the base is an alkali metal salt of a weak acid.

12. A process, as in claim 11, wherein the base is carbonate of sodium.

13. A process, as in claim 10, wherein the base is sodium hydroxide.

14. A process, as in claim 8, wherein the high consistency pulp has a consistency between about 15 and about 50.

15. In a process of bleaching a cellulosic pulp which comprises:

- treating a chemical cellulosic pulp to solubilize ligneous impurities, and
- extracting the resultant pulp with aqueous base, the improvement which comprises,
- contacting the resultant pulp at high consistency and in the form of fluffed or shredded fibers or fiber aggregates with a gaseous medium wherein the active contacting component consists essentially of gaseous chlorine and the pH of the pulp is maintained between about 7 and about 10 during the gaseous chlorine contacting stage, thereby effecting bleaching of said pulp,
- extracting the resultant pulp with aqueous base,

11

e. contacting the resultant pulp at high consistency and in the form of fluffed or shredded fibers or fiber aggregates with a gaseous medium wherein the active contacting component consists essentially of gaseous chlorine wherein the amount of gaseous chlorine is an effective bleaching inducing amount of chlorine which is about 1% or less by weight based on the weight of moisture-free cellulosic pulp, thereby effecting bleaching of said pulp.

16. A process for bleaching a pretreated or pre-bleached and extracted fibrous cellulosic pulp having a Permanganate Number of about 5 or less which comprises contacting said pulp at high consistency and in the form of fluffed or shredded fibers or fiber aggregates with a gaseous medium wherein the active contacting component consists essentially of gaseous chlorine wherein the amount of gaseous chlorine is an effective bleaching inducing amount of chlorine which is about 1% or less by weight based on the weight of moisture-free cellulosic pulp, thereby effecting bleaching of said pulp.

12

gates with a gaseous medium wherein the active contacting component consists essentially of gaseous chlorine wherein the amount of gaseous chlorine is an effective bleaching inducing amount of chlorine which is about 1% or less by weight based on the weight of moisture-free cellulosic pulp and the pH of the pulp is maintained between about 7 and about 10 during the gaseous chlorine contacting, thereby effecting a bleaching of said pulp.

17. A process, as in claim 16, wherein the high consistency pulp has a consistency between about 15 and about 50.

\* \* \* \* \*

15

20

25

30

35

40

45

50

55

60

65